

Jan. 1, 1946.

J. MCORLTY

2,391,995

ELECTRICAL HEATING ELEMENT

Filed Aug. 6, 1945



JOSEPH MCORLTY

INVENTOR

BY Freeman, Albrecht and Williams

ATTORNEYS

## UNITED STATES PATENT OFFICE

2,391,995

## ELECTRICAL HEATING ELEMENT

Joseph McOrlly, Wilkinsburg, Pa., assignor to  
 Edwin L. Wiegand Company, Pittsburgh, Pa.,  
 a corporation of Pennsylvania

Application August 6, 1945, Serial No. 609,135

9 Claims. (Cl. 201—64)

My invention relates to embedded-resistor electric heating elements, and the principal object of my invention is to provide new and improved elements of that type.

This application is a continuation in part of my copending application Serial Number 346,847, filed July 22, 1940.

In the drawing accompanying this specification and forming a part of this application, as in the drawing forming a part of said application 10 346,847, I have shown, for purposes of illustration, various types of electric heating elements in which my invention may be embodied, and therein:

Figure 1 is a plan view of a ring type heating 15 element,

Figures 2 and 3 are sections on the lines 2—2 and 3—3 respectively of Figure 1.

Figure 4 is a plan view of a strip type heating element,

Figure 5 is a fragmentary longitudinal section of a tubular type heating element,

Figure 6 is a section on the line 6—6 of Figure 5,

Figure 7 is a plan view of a cast plate type of heating element, and—

Figure 8 is a section on the line 8—8 of Figure 7.

The ring type heating element shown in Figures 1 through 3 comprises an annular sheet metal sheath 10, a resistor 11 disposed within the sheath 10, and embedding material 12 serving both to insulate the resistor 11 electrically and also to conduct the heat from the resistor 11 to the sheath 10.

As here shown the resistor 11 consists of resistance wire wound helically, and the sheath 10 comprises an annular sheet metal channel 13 providing an annular plane face 14, and a sheet metal cover plate 15 held in position by the turned-over margins 16 of the channel 13 and provided with an embossed portion 24 containing apertures 21 for the passage of the shanks 18 of terminal studs 17 to which the ends 25 and 26 of the resistor 11 are electrically connected.

In the present embodiment the studs 17 are provided with heads 18 of suitable form, and the ends 25 and 26 of the resistor 11 encircle the shanks 18 of the studs 17 below these heads 18, also the studs 17 are spaced circumferentially, and the intermediate helical portion of the resistor 11 is disposed in a plurality of passes each substantially concentric with the sheath 10, as shown particularly in Figure 1.

Likewise each of the shanks 18 is encircled by inner and outer mica washers 22 and 23 disposed respectively interiorly and exteriorly of the cover plate 15, and the outer end of each of the shanks 18 is screw threaded to receive a cooperating nut

20, whereby the studs 17 are mounted electrically insulated from the cover plate 15 and sheath 10.

One way of constructing a heating element of the type shown in Figures 1 through 3 comprises the following: The resistor 11 and terminal studs 17 are mounted on a suitable form (not shown) analogous to the form shown in Wiegand Patent 1,183,347, but of course of a shape and size to accord with the channel 13. Coordinately there is placed in the channel 13 a proper depth of embedding material, which whether or not it includes bonding material, in any event is in a plastic, plastoid, or impressionable condition. Then the form carrying the resistor 11 is introduced into the channel 13 under pressure, resulting in embedding the resistor 11 in the embedding material and compacting the embedding material in the lower part of the channel 13. Following this the form is withdrawn, leaving the resistor 11 embedded in the material compacted in the channel 13. Then additional embedding material is introduced into the channel 13, again to a proper depth, and likewise compacted, and thereafter the cover plate 15 is added, and the margins 16 of the channel 13 are turned over, and hold the cover plate 15 in place and the element assembled. Additionally, the element may be subjected to various drying or baking steps or both, at any stage of the manufacture, or as a final treatment, and also to other pressing operations, as may be desired.

The strip type heating element shown in Figure 4, is similar to the ring type heating element shown in Figures 1 through 3, but is of elongated rectilinear form, including the sheath 10a, the channel 13a, and the cover plate 15a. The terminals 17a are here shown as at opposite ends, and the resistor 11a as composed of three passes. The extremities of the sheath 10a contain no insulating material, but are pressed together, to close the ends of the sheath. One way of making these elements is by generally the same process described for the ring type elements shown in Figures 1 through 3.

The tubular type heating element shown in Figures 5 and 6, comprises a seamless tubular metallic sheath 27 in which is disposed a resistor 28 embedded in embedding material 29. The resistor 28 may be of any suitable form, and may be connected at its ends to terminal rods 30, one of which is shown, or to terminals of any other suitable and desired form and construction. Each end of the tubular sheath 27 may be closed by an end wall or plug 31, which may be of mica or other suitable insulation, and may be provided with an aperture through which the respective terminal extends, and within which the terminal may be sealed. Also the end of the sheath 27 may have a portion 32 crimped over the end wall or plug 31. One way of making this

type of element is by suitably disposing the resistor 28 within the sheath 27, and then adding embedding material to embed the resistor, and preferably compacting the embedding material, in any suitable manner.

The cast plate type of heating element shown in Figures 7 and 8, comprises a sheath consisting of a cast metal plate 38 provided with grooving 39 in which is disposed a resistor 38 embedded in embedding material 36 and connected to terminals 37 projecting beyond the embedding material 36. One way of making this type of element is by generally the same process described for the ring type elements shown in Figures 1 through 3, of course omitting the steps of adding the cover plate and turning over the margins of the channel.

In electric heating elements of the types herein shown and above described, and likewise in embedded-resistor electric heating elements of various other types, previously it has been customary to employ as the embedding material a composition comprising essentially granular refractory material, for example, zircon, alumina, sillimanite, or a mixture, and bonding material, for example, 20 clay or kaolin, and such compositions have been acceptable, and still are acceptable, under low requirements of performance.

However, by way of example, ring type elements as shown in Figures 1 through 3, and also cast plate type elements as shown in Figures 7 and 8, are of a form inherently highly suitable for electric hot plate units and electric range top units. On the other hand, for such units to be satisfactory for that purpose, the embedding material must be high heat conducting, low electrical leakage, and suitable for operation, at red heat or above.

According to my invention, this may be accomplished by eliminating the previous bonding material, and including a quantity of talc. Further, contrary to what might be expected, the talc not only provides the desirable workability of the composition in and during the making of the element, but apparently serves also to knit the granular material, at least sufficiently to hold the resistor and the terminals in position, and on the other hand, within limits, does not objectionably reduce the thermal conductivity, at least in terms of ability of the embedding to conduct the heat from the resistor.

Of course the elimination of the previous bonding material, and to some extent the inclusion of the talc, result in very great enhancement of the electrical values, including very large decrease in the electrical leakage.

However, at least on the basis of what I have thus far been able to accomplish, to produce an embedding capable of holding the resistor and the terminals in position, the talc must be present in an amount not less than approximately 3%, and to avoid objectionable decrease in the ability of the embedding to conduct the heat from the resistor, the talc must not be included in an amount more than approximately 40%, and preferably should not be included in amount more than approximately 30%, by weight.

On the other hand, at least according to present indications, with the inclusion of talc, seemingly there is no disadvantage, and apparently some advantage, at least in some instances, in including also a quantity of the previous bonding material.

For example, the inclusion of a quantity of the previous embedding material generally will result

in an embedding additionally effective to hold the resistor and the terminals in position, and additionally effective to conduct the heat from the resistor, and at the same time, apparently by reason of dispersion of the previous bonding material by the talc, will not objectionably increase the electrical leakage, or objectionably impair any of the other electrical values.

However, at least on the basis of what I have thus far been able to accomplish, the previous bonding material, if it is included, should not be present in an amount more than approximately 20%, and preferably should not be present in an amount more than approximately 15%, by weight.

By way of example, an excellent embedding material results from a composition consisting of approximately 76% granular material, 17% talc, and 7% bonding material, by weight, the granular material being zircon, and the bonding material being kaolin.

This composition, in a suitably moist condition, may be introduced into the sheath, and the resistor embedded therein, and the composition compacted, as above described, and when dried and baked produces a firm cake, of low electrical leakage and high thermal conductivity, and entirely adequate to retain the resistor in position.

Heating elements employing this embedding may be operated safely, for example, immersed in liquid, at watt densities of 50 to 60 watts per square inch of heating surface. The thickness of the embedding material between the passes of the resistor, and between the resistor and the sheath, may be small, for example, as little as approximately 0.07 to 0.09 of an inch. With the element operated at temperatures of the order of 1200° to 1600° Fahrenheit, the electrical leakage nevertheless is very small, and only a fraction of the electrical leakage in a similar element employing the previous embedding material and operated at only 30 to 40 watts per square inch and therefore at materially lower temperature.

Therefore an embedding of the above composition is particularly suitable for electric hot plate units and electric range top units, intended for operation at high temperature, and nevertheless limited to very low electrical leakage.

In another instance, in which it is permissible that the embedding be less firm, I have found successful a similar composition consisting of approximately 72% granular material, 21% talc, and 7% bonding material, resulting in an embedding which may be referred to as articulating, in that to a degree it may be likened to what is known as flexible sandstone. Apparently the grains of the granular material are embedded in a matrix of the talc and bonding material, and the embedding can expand, contract, and bend, without showing cracks.

Therefore this composition is particularly advantageous in instances involving relatively long length of embedding and aggravated problems of contraction and expansion, for example, in cast plate type heating elements as shown in Figures 7 and 8.

Other particular compositions are, including bonding material, approximately 76% granular material, 6% talc, and 18% bonding material, and approximately 60% granular material, 35% talc, and 5% bonding material, and not including bonding material, approximately 95% granular material and 5% talc, approximately 80% granular material and 20% talc, and approximately 65% granular material and 35% talc, by weight, and

in these also the granular material may be zircon, and the bonding material may be kaolin.

When zircon is used, in many instances I prefer natural grain zircon, usually obtained screened —60 mesh, and containing very little if any —200 mesh, the greater part lying between 100 mesh and 120 mesh. On the other hand, in some instances I prefer that the granular material be wholly or partially ground zircon, screened —400 mesh.

For the bonding material, in most instances I prefer kaolin, but I may use ball clay, or semi-ball clay, either alone or in conjunction with kaolin. However, apparently it is preferable that the alkali content of the kaolin or clay be not more than approximately 0.25%, that the calcium oxide content also should be low, that no chemical be used in washing the kaolin or clay, either basic or acid, to avoid absorption, and that the kaolin or clay be dried and pulverized to a substantially uniform fineness of air-float size.

For the talc, apparently it is desirable to use an electrical grade of talc, and apparently it is preferable that the talc be low in lime and alkali salts or other impurities, and white-burning. In this connection it is to be understood that the term talc is herein used generically, and under proper circumstances includes for example soapstone and steatite.

In pressing the composition I may use pressures as low as 500 pounds or less, up to 10 to 15 tons or more, per square inch, depending on the circumstances in the particular instance, and likewise drying may be at room temperature, or above or below, and baking may be at a temperature, for example, of the order of 1200° Fahrenheit, or higher or lower.

Further, as will be understood by those skilled in the art, the four types of heating units shown in the drawing are illustrative only, and also, while reference has been made to embedding material having high heat conductivity and low electrical leakage and suitable for operation at red heat, of course this merely is definitive of the embedding, and the temperature at which the element or embedding actually is operated, is immaterial.

Accordingly, it will be obvious to those skilled in the art, that I have accomplished at least the principal object of my invention, and on the other hand, that the disclosure herein is illustrative only, and that my invention is not limited thereto.

Now, therefore, I claim as follows:

1. An embedded-resistor electric heating element comprising embedding having high heat conductivity and low electrical leakage and suitable for operation at red heat, consisting of material compacted under pressure, comprising granular refractory material of high heat conductivity and low electrical leakage, and comprising also talc, the talc constituting approximately 3% to approximately 40%, and the granular material and talc constituting at least approximately 80%, by weight.

2. An embedded-resistor electric heating element comprising embedding having high heat conductivity and low electrical leakage and suitable for operation at red heat, consisting of material compacted under pressure, and comprising talc approximately 3% to approximately 40%, by weight, and the remainder substantially entirely granular refractory material of high heat conductivity and low electrical leakage.

3. An embedded-resistor electric heating ele-

ment comprising embedding having high heat conductivity and low electrical leakage and suitable for operation at red heat, consisting of material compacted under pressure, comprising granular refractory material of high heat conductivity and low electrical leakage, and comprising also bonding material and talc, the talc constituting approximately 3% to approximately 40%, the bonding material constituting not more than approximately 20%, and the granular material and talc constituting at least approximately 80%, by weight.

4. An embedded-resistor electric heating element comprising embedding having high heat conductivity and low electrical leakage and suitable for operation at red heat, consisting of material compacted under pressure, comprising granular refractory material of high heat conductivity and low electrical leakage, and comprising also talc, the talc constituting approximately 3% to approximately 30%, and the granular material and talc constituting at least approximately 85%, by weight.

5. An embedded-resistor electric heating element comprising embedding having high heat conductivity and low electrical leakage and suitable for operation at red heat, consisting of material compacted under pressure, and comprising talc approximately 3% to approximately 30%, by weight, and the remainder substantially entirely granular refractory material of high heat conductivity and low electrical leakage.

6. An embedded-resistor electric heating element comprising embedding having high heat conductivity and low electrical leakage and suitable for operation at red heat, consisting of material compacted under pressure, comprising granular refractory material of high heat conductivity and low electrical leakage, and comprising also bonding material and talc, the talc constituting approximately 3% to approximately 30%, the bonding material constituting not more than approximately 15%, and the granular material and talc constituting at least approximately 85%, by weight.

7. An embedded-resistor electric heating element comprising embedding having high heat conductivity and low electrical leakage and suitable for operation at red heat, consisting of material compacted under pressure, and comprising granular refractory material of high heat conductivity and low electrical leakage, approximately 75%, and talc, approximately 7%, and bonding material, approximately 18%.

8. An embedded-resistor electric heating element comprising embedding having high heat conductivity and low electrical leakage and suitable for operation at red heat, consisting of material compacted under pressure, and comprising granular refractory material of high heat conductivity and low electrical leakage, approximately 76%, and talc, approximately 17%, and bonding material, approximately 7%.

9. An embedded-resistor electric heating element comprising embedding having high heat conductivity and low electrical leakage and suitable for operation at red heat, consisting of material compacted under pressure, and comprising granular refractory material of high heat conductivity and low electrical leakage, approximately 60%, and talc, approximately 35%, and bonding material, approximately 5%.

JOSEPH MCORRY.